



US011946015B2

(12) **United States Patent**  
**Kaneko**

(10) **Patent No.:** **US 11,946,015 B2**  
(45) **Date of Patent:** **Apr. 2, 2024**

(54) **WATER GLYCOL-BASED HYDRAULIC FLUID**

(71) Applicant: **SHELL OIL COMPANY**, Houston, TX (US)

(72) Inventor: **Hiroshi Kaneko**, Tokyo (JP)

(73) Assignee: **SHELL USA, INC.**, Houston, TX (US)

(\*) Notice: Subject to any disclaimer, the term of this patent is extended or adjusted under 35 U.S.C. 154(b) by 0 days.

(21) Appl. No.: **17/910,879**

(22) PCT Filed: **Apr. 1, 2021**

(86) PCT No.: **PCT/EP2021/058650**

§ 371 (c)(1),

(2) Date: **Sep. 12, 2022**

(87) PCT Pub. No.: **WO2021/198435**

PCT Pub. Date: **Oct. 7, 2021**

(65) **Prior Publication Data**

US 2023/0105327 A1 Apr. 6, 2023

(30) **Foreign Application Priority Data**

Apr. 3, 2020 (JP) 2020-067577

(51) **Int. Cl.**

**C10M 173/02** (2006.01)  
**C10N 30/06** (2006.01)

(52) **U.S. Cl.**

CPC ..... **C10M 173/02** (2013.01); **C10M 2201/02** (2013.01); **C10M 2201/062** (2013.01); **C10N 2030/06** (2013.01)

(58) **Field of Classification Search**

CPC ..... C10M 173/02; C10M 2201/02; C10M 2201/062; C10M 2207/0225; C10M 2207/122; C10M 2207/126; C10M 2207/127; C10M 2207/129; C10M 2207/22; C10N 2030/06; C10N 2040/08

See application file for complete search history.

(56) **References Cited**

**U.S. PATENT DOCUMENTS**

|                 |   |         |                 |       |             |
|-----------------|---|---------|-----------------|-------|-------------|
| 3,580,847 A     | * | 5/1971  | Boehmer         | ..... | C10M 173/02 |
|                 |   |         |                 |       | 252/78.3    |
| 3,992,312 A     | * | 11/1976 | Genjida         | ..... | C10M 173/02 |
|                 |   |         |                 |       | 252/77      |
| 9,695,380 B2    |   | 7/2017  | Greaves         |       |             |
| 2009/0242858 A1 |   | 10/2009 | Palmerio et al. |       |             |

**FOREIGN PATENT DOCUMENTS**

|    |              |         |
|----|--------------|---------|
| JP | H04106196 A  | 4/1992  |
| JP | H06279780 A  | 10/1994 |
| JP | H07233391 A  | 9/1995  |
| JP | H08143888 A  | 6/1996  |
| JP | 2646308 B2   | 8/1997  |
| JP | H09208985 A  | 8/1997  |
| JP | 2001107075 A | 4/2001  |
| JP | 3233490 B2   | 11/2001 |
| JP | 2007246684 A | 9/2007  |
| JP | 2011241270 A | 12/2011 |
| JP | 2012224795 A | 11/2012 |
| JP | 2014051650 A | 3/2014  |
| JP | 2016050217 A | 4/2016  |

**OTHER PUBLICATIONS**

International Search Report and Written Opinion received for PCT Patent Application No. PCT/EP2021/058650, dated Jun. 24, 2021, 9 pages.

Office Action Received for Chinese Application No. 202180026623, 4, dated Feb. 7, 2023, 14 Pages (7 Pages of English Translation and 7 Pages of Official Copy).

Office Action Received for Japanese Application No. 2020-067577, dated Jan. 23, 2024, 07 Pages (03 Pages of English Translation and 04 Pages of Official Copy).

\* cited by examiner

*Primary Examiner* — Cephia D Toomer

(74) *Attorney, Agent, or Firm* — SHELL USA, INC.

**ABSTRACT**

The present invention provides a water-glycol hydraulic fluid comprising 0.3-0.6% by mass in total of fatty acid sodium salt and/or fatty acid, and 0.3-0.6% by mass of dimerized fatty acid. The water-glycol hydraulic fluid also comprises 20-60% by mass water, 20-60% by mass glycol, 0.01-0.06% by mass alkali hydroxide compound selected from potassium hydroxide and/or sodium hydroxide, and 1.0-5.0% by mass alkanolamine.

**3 Claims, No Drawings**

## WATER GLYCOL-BASED HYDRAULIC FLUID

### CROSS REFERENCE TO RELATED APPLICATIONS

This is a National stage application of International application No PCT/EP2021/058650, filed 1 Apr. 2021, which claims priority of JP application No. 2020-067577, filed 3 Apr. 2020 which is incorporated herein by reference in its entirety.

### TECHNICAL FIELD OF THE INVENTION

The present invention relates to an improved water-glycol hydraulic fluid used as a fire-resistant hydraulic fluid.

### BACKGROUND OF THE INVENTION

Hydraulic equipment is used widely in industry, where it contributes to improvements in productivity, and is also used widely by the general public. The hydraulic fluid is used as a medium for transmitting power in hydraulic equipment. Hydraulic fluids are widely used in hydraulic equipment, and hydraulic fluids containing a mineral oil-based base oil are commonly used.

However, hydraulic equipment used in mechanical equipment such as die casting machinery, forging presses, steel-making equipment used in the steel industry where fire resistance is required, and hydraulic equipment used in amusement park equipment and stage equipment in indoor facilities where fire safety is important, cannot use petroleum-based hydraulic oils, which lack heat resistance, so flame-retardant water-based hydraulic fluids are used.

When a water-based water-glycol hydraulic fluid is used as a water-based hydraulic fluid, good wear resistance and lubricity are required so that hydraulic operations can be performed smoothly and the service life of hydraulic equipment can be extended. Therefore, water-based hydraulic fluid compositions obtained by, for example, adding a polyoxalkylene glycol diether compound having a specific structure, a polyoxalkylene glycol monoether compound, a polyoxypropylene glycol monoether compound, and a fatty acid salt to water are used to improve performance in terms of lubricity and wear resistance (see JP3233490 B2).

Some water-glycol hydraulic fluids also include a small amount of a neutralization product of glycerol borate and base obtained by reacting glycerol with boric anhydride or boron trichloride, such as in JP2646308 B2. Other water-glycol hydraulic fluids contain a water-soluble polyether having a specific structure derived from a water-soluble polyoxalkylene polyol and glycidyl ether, for example in JP H07-233391 A.

It is an object of the present invention to obtain a water-glycol hydraulic fluid having greatly improved wear resistance and good performance without impairing any other type of performance provided by water-glycol hydraulic fluid by including specific additives in the water-glycol hydraulic fluid.

### SUMMARY OF THE INVENTION

The present invention provides a water-glycol hydraulic fluid containing 20-60% by mass water and 20-60% by mass glycol, with the remainder being, for example, a fatty acid-based lubricant, alkaline hydroxide compound, thickener, rust inhibitor, anticorrosive, and antifoaming agent to

bring the total to 100% by mass. As a result of extensive research and development conducted to solve this problem, the present inventor and others discovered that use of a small amount of a sodium salt of a specific fatty acid could significantly improve the wear resistance of a water-glycol hydraulic fluid. The present invention is based on this discovery. Specifically, the present invention is a water-glycol hydraulic fluid containing a fatty acid having from 4 to 18 carbon atoms, a sodium salt of a fatty acid having 4 to 18 carbon atoms, and a dimerized fatty acid. This fatty acid or sodium salt of a fatty acid can be used alone or in combination for a total amount of 0.3 to 0.6% by mass, and the dimerized fatty acid can be used in an amount of 0.3 to 0.6% by mass.

### DETAILED DESCRIPTION OF THE INVENTION

The present invention can readily obtain an easy-to-use water-glycol hydraulic fluid having greatly improved wear resistance while maintaining and not impairing any other type of performance provided by water-glycol hydraulic fluid by including small amounts of a specific fatty acid and/or sodium salt of a specific fatty acid and a dimerized fatty acid in the water-glycol hydraulic fluid.

These fatty acids are saturated fatty acids having four or more carbon atoms. Examples include butyric acid, valeric acid, caproic acid, enanthic acid, caprylic acid, pelargonic acid, capric acid, undecylic acid, lauric acid, tridecyllic acid, myristic acid, pentadecyllic acid, palmitic acid, margaric acid, stearic acid, nonadecyllic acid, and arachidic acid. These fatty acids can also be unsaturated fatty acids such as oleic acid, linoleic acid, and linolenic acid.

Examples of fatty acid sodium salts include sodium butyrate, sodium valerate, sodium caproate, sodium enanthate, sodium caprilate, sodium pelargonate, sodium caprate, sodium undecylate, sodium laurate, sodium tridecylate, sodium myristate, sodium pentadecylate, sodium palmitate, sodium margarate, sodium stearate, sodium nonadesilate, sodium arachidate, sodium oleate, sodium linoleate, and sodium linolenate. These fatty acids and sodium salts of fatty acid are used alone or in combination in a total amount of 0.3 to 0.6% by mass, preferably 0.35 to 0.50% by mass, based on the total mass of the composition. Note that potassium salts, which are the same type of alkali metal salt, are not preferred. Use of sodium salts is preferred to potassium salts in terms of thermal stability.

Dimerized fatty acids are liquid fatty acids containing a dibasic acid of a C36 dicarboxylic acid produced by dimerization of a C18 unsaturated fatty acid containing a vegetable fat or oil as a main component, but also a monobasic acid and a tribasic acid. These dimerized fatty acids are included in an amount of 0.3 to 0.6% by mass, preferably 0.35 to 0.50% by mass, based on the total mass of the composition.

A water-glycol-based hydraulic fluid of the present invention contains 20-60% by mass glycol, 0.01-0.06% by mass alkali hydroxide compound selected from potassium hydroxide and/or sodium hydroxide, and 1.0-5.0% by mass of alkanolamine. It also contains a fatty acid sodium salt or fatty acid having from 4 to 12 carbon atoms and a dimerized fatty acid. The water-glycol-based hydraulic solution contains water. The amount of water is 20-60% by mass, more preferably 30-50% by mass, and the amount of water added brings the total amount of hydraulic fluid composition to 100% by mass.



The test results are shown in Table 1 and Table 2.

TABLE 1

|                           | Ex. 1   | Ex. 2   | Ex. 3   |
|---------------------------|---------|---------|---------|
| Sodium laurate            | 0.450   | 0.200   |         |
| Lauric acid               |         | 0.225   | 0.400   |
| Dimerized fatty acid      | 0.400   | 0.400   | 0.400   |
| Alkanolamine              | 1.900   | 1.900   | 1.900   |
| Glycol                    | 38.628  | 38.653  | 38.678  |
| Alkali hydroxide compound | 0.060   | 0.060   | 0.060   |
| Thickener                 | 16.100  | 16.100  | 16.100  |
| Other additives           | 0.620   | 0.620   | 0.620   |
| Water                     | 41.842  | 41.842  | 41.842  |
| Total                     | 100.000 | 100.000 | 100.000 |
| Wear mark diameter (mm)   | 0.46    | 0.49    | 0.52    |
|                           | ○       | ○       | ○       |
| Total amount of wear (mg) | 45.3    | —       | 59.2    |

TABLE 2

|                           | Comp.<br>Ex. 1 | Comp.<br>Ex. 2 | Comp.<br>Ex. 3 |
|---------------------------|----------------|----------------|----------------|
| Lauric acid               | 0.200          |                | 0.400          |
| Dimerized fatty acid      | 0.200          | 0.400          |                |
| Alkanolamine              | 1.900          | 1.900          | 1.900          |
| Glycol                    | 39.078         | 39.078         | 39.078         |
| Alkali hydroxide compound | 0.060          | 0.060          | 0.060          |
| Thickener                 | 16.100         | 16.100         | 16.100         |
| Other additives           | 0.620          | 0.620          | 0.620          |
| Water                     | 41.842         | 41.842         | 41.842         |
| Total                     | 100.000        | 100.000        | 100.000        |
| Wear mark diameter (mm)   | 0.78           | 0.87           | 0.88           |
|                           | x              | x              | x              |

As shown in Table 1, in Example 1, which contained a fatty acid sodium salt, the wear mark diameter in the Shell four ball lubricant test was a low 0.46 mm, and the total amount of wear after 250 hours in the lubricity pump test was 45.3 mg. These results indicate superior lubricity performance. In Example 2, which contained less fatty acid sodium salt and the same fatty acid, the wear mark diameter in the Shell four ball lubricant test was 0.49 mm, which is a good result. In Example 3, which contained only a fatty acid, the wear mark diameter in the Shell four ball lubricant test was a low 0.52 mm, and the total amount of wear in the lubricity pump test was 59.2 mg. These results indicate superior lubricity performance.

As shown in Table 2, Comparative Example 1, which did not contain a fatty acid sodium salt and which included less fatty acid and dimerized fatty acid, failed in terms of the wear mark diameter. Comparative Example 2, which contained neither a fatty acid nor a fatty acid sodium salt, also failed. Comparative Example 3, which did not contain a dimerized fatty acid, failed as well. Because Comparative Examples 1-3 all failed in terms of the wear mark diameter, measurement of the total amount of wear in the lubricity pump test was omitted.

We claim:

1. A water-glycol hydraulic fluid comprising 20-60% by mass water, 20-60% by mass glycol, 0.01-0.06% by mass alkali hydroxide compound selected from potassium hydroxide and/or sodium hydroxide, 1.0-5.0% by mass alkanolamine, 0.3-0.6% by mass in total of fatty acid sodium salt and/or fatty acid having from 4 to 18 carbon atoms, and 0.3-0.6% by mass of dimerized fatty acid.

2. The water-glycol hydraulic fluid according to claim 1, wherein the fatty acid sodium salt is sodium laurate having 12 carbon atoms.

3. The water-glycol hydraulic fluid according to claim 1, wherein the fatty acid is lauric acid having 12 carbon atoms.

\* \* \* \* \*